# EUROPEAN PATENT APPLICATION

(11) **EP 1 883 092 A2**
(43) Date of publication of application: **30.01.2008**
(21) Application number: 07252827.6
(22) Date of filing: 17.07.2007
(51) Int. Cl.: H01J 17/04, H01J 17/49, H01J 9/20

(54) **Plasma display panel and method for manufacturing the same**

(30) Priority: 28.07.2006 KR 20060071600; 28.07.2006 KR 20060071601; 29.01.2007 KR 20070008805
(71) Applicant: LG Electronics Inc., Seoul, 150-721 (KR)
(72) Inventor: Kim, Bo Hyun, Seocho-Gu, Seoul 137-724 (KR); Park, Min Soo, Seocho-Gu, Seoul 137-724 (KR); Park, Deok Hai, Seocho-Gu, Seoul 137-724 (KR); Ryu, Byung Gil, Seocho-Gu, Seoul 137-724 (KR); Kim, Young Sung, Seocho-Gu, Seoul 137-724 (KR); Song, Moon Bong, Seocho-Gu, Seoul 137-724, (KR); Cho, Won Ki, Seocho-Gu, Seoul 137-724 (KR)
(74) Representative: Camp, Ronald

(57) **Abstract**

A protective layer of a plasma display panel is disclosed. In the plasma display panel including a first panel (70) and a second panel (10) arranged to face each other while interposing barrier ribs (40) therebetween, the plasma display panel further includes a first protective (100a) layer formed on a dielectric layer (90) of the first panel, and a second protective layer (100b) formed on the first protective layer and containing a metallic oxide having a maximum cathode ray luminescence value within a wavelength region of 300 to 500 nanometers.

## Description

### BACKGROUND OF THE INVENTION

### Field of the Invention

The present invention relates to a display apparatus. It more particularly relates to a protective layer and a method for manufacturing the same.

### Discussion of the Related Art

With the advent of the multimedia age, there is rising a demand for the appearance of a more delicate and greater display apparatus capable of representing colors close to natural colors. Since a current cathode ray tube (CRT) has a limit to construct a large-size screen of 40 inches or more, a liquid crystal display (LCD), a plasma display panel (PDP), a projection television (TV), etc. are rapidly growing for the expansion of their use purposes to the field of a high definition image.

A plasma display panel includes a lower panel having address electrodes, an upper panel having sustain electrode pairs, and discharge cells defined as barrier ribs, a phosphor being applied inside each discharge cell. Here, each of the discharge cells is filled with a primary discharge gas, such as neon, helium, a mixed gas of neon and helium, or the like, and an inert gas containing a small amount of xenon. If an electric discharge occurs in a discharge space between the upper panel and the lower panel, vacuum ultraviolet rays are produced and are irradiated onto the phosphor of each discharge cell, to produce visible rays. With the visible rays, an image is displayed on a screen.

Both the upper panel and the lower panel of the plasma display panel are formed with dielectric layers, respectively, to protect the sustain electrode pairs and the address electrodes. However, while an electric discharge occurs in the plasma display panel, the upper dielectric layer formed at the upper panel becomes worn and disappears due to the shock caused by positive ions. Therefore, the electrodes of the upper panel have the risk of becoming short circuited by metallic element such as sodium, etc.

To solve the above described problem, a protective layer is formed on the upper dielectric layer provided at the upper panel. The protective layer is formed, for example, as a coating layer of magnesium oxide (MgO) having high resistance against the shock caused by positive ions and a high discharge coefficient of secondary electrons. With the formation of the protective layer, the drive voltage required for the plasma display panel can be lowered. Such a low drive voltage has advantages of reducing the consumption of electricity by the plasma display panel and providing the plasma display panel with improved brightness and discharge efficiency, etc.

However, the protective layer of the above described conventional plasma display panel has the following problems.

When the protective layer is made of magnesium oxide, foreign substances may be contained in the protective layer, thereby causing a deterioration in jitter characteristics. Therefore, it is necessary to provide a homogeneous protective layer for preventing a deterioration in jitter characteristics. However, the protective layer of the conventional plasma display panel cannot be free from foreign substances in a surface thereof. Furthermore, in the protective layer containing the foreign substances, fine cracks may occur at the surface of the protective layer due to shock caused by plasma particles. The cracks result in a reduction in the lifespan of the protective layer, and may reduce the number of secondary electrons discharged from the protective layer during an opposed discharge.

When the protective layer is made only of magnesium oxide, although the protective layer is able to increase the discharge coefficient of secondary electrons to some extent, the increase of the discharge coefficient has a limit, and the resulting plasma display panel has problems of a high drive voltage and a low efficiency.

### SUMMARY OF THE INVENTION

Accordingly, the present invention is directed to an improved plasma display panel and a method for manufacturing the same.

Additional advantages and features of the invention will be set forth in part in the description which follows and in part will become apparent to those having ordinary skill in the art upon examination of the following or may be learned from practice of the invention. The advantages of the invention may be realized and attained by the structure particularly pointed out in the written description and claims hereof as well as the appended drawings.

In accordance with a first aspect of the invention, a plasma display panel comprising a first panel and a second panel arranged to face each other while interposing barrier ribs therebetween, further comprises: a first protective layer formed on a dielectric layer of the first panel; and a second protective layer formed on the first protective layer and containing a metallic oxide having a maximum cathode ray luminescence value within a wavelength region of 300 to 500 nanometers.

In accordance with another aspect of the present invention, there is provided a method for manufacturing a plasma display panel comprising: depositing a first protective layer on a dielectric layer of a first panel; and depositing a second protective layer on the first protective layer, the second protective layer containing a single-crystal metallic oxide having a maximum cathode ray luminescence value within a wavelength region of 300 to 500 nanometers.

In accordance with yet another aspect of the present invention, there is provided a method for manufacturing magnesium oxide comprising: preparing magnesium gas; and supplying the magnesium gas with oxygen gas and argon gas, to form a magnesium oxide single crystal.

It is to be understood that both the foregoing general description and the following detailed description of the present invention are exemplary and explanatory and are intended to provide further explanation of the invention as claimed.

### BRIEF DESCRIPTION OF THE DRAWINGS

The accompanying drawings, which are included to provide a further understanding of the invention and are incorporated in and constitute a part of this application, illustrate embodiment(s) of the invention and together with the description serve to explain the principle of the invention by way of non-limiting example. In the drawings:

FIG. 1 is a view illustrating an embodiment of the configuration of protective layers included in a plasma display panel according to the present invention;

FIG. 2 is a perspective view illustrating the configuration of discharge cells included in the plasma display panel according to an embodiment of the present invention;

FIGs. 3A and 3B are graphs illustrating a surface discharge voltage and an opposed discharge voltage of the plasma display panel according to the present invention;

FIG. 4A is a graph illustrating the jitter characteristics of the plasma display panel according to the present invention;

FIG. 4B is a graph illustrating the cathode ray luminescence characteristics of a metallic oxide constituting the protective layer of the plasma display panel according to the present invention;

FIG. 5 is a view illustrating an embodiment of a chemical vapor deposition apparatus according to the present invention; and

FIG. 6 is a flow chart illustrating an embodiment of a method for manufacturing a second protective layer of a plasma display panel according to the present invention.

### DETAILED DESCRIPTION OF THE INVENTION

Reference will now be made in detail to the preferred embodiments of the present invention, examples of which are illustrated in the accompanying drawings. Wherever possible, the same reference numbers will be used throughout the drawings to refer to the same or like parts.

FIG. 1 is a view illustrating an embodiment of the configuration of protective layers included in a plasma display panel according to the present invention. Now, the preferred embodiment of the protective layers included in the plasma display panel according to the present invention will be described with reference to FIG. 1.

A first protective layer 100a is formed on a dielectric layer (not shown). The first protective layer 100a is made of magnesium oxide, and additionally, a dopant may be contained in the first protective layer 100a. The dopant has the function of improving the discharge characteristics of secondary electrons included in the protective layer and reducing the delay of a discharge. The dopant may be selected from the group consisting of aluminum (Al), chrome (Cr), hydrogen (H₂), silicon (Si), scandium (Sc), and gadolinium (Gd). The first protective layer 100a may have a thickness of 100 to 1,000 nanometers. Preferably, to reduce a jitter value to the maximum extent, the dopant contained in the first protective layer 100a is in an amount of 20 to 500 parts per million (ppm).

A second protective layer 100b is formed on the first protective layer 100a. The second protective layer 100b may contain a metallic oxide. Here, the metallic oxide has a feature of having a maximum cathode ray luminescence value within a wavelength region of 300 to 500 nanometers. Also, the metallic oxide has a feature of being produced by supplying a gas-phase metallic element with 2 to 20 sccm of oxygen and 0 to 18 sccm of argon. The reason why the second protective layer 100b made of a metallic oxide is additionally provided is that the first protective layer 100a has a weak point in jitter characteristics and discharge efficiency although it protects a dielectric layer from shock caused by positive ions. The second protective layer 100b may have a thickness of 100 to 1,500 nanometers. The metallic oxide may have a particle size of 50 to 1,000 nanometers.

Here, the metallic oxide in the second protective layer 100b may be a single-crystal magnesium oxide powder or an alkali or alkaline-earth metallic oxide. It will be appreciated from the following Table 1 that the protective layer containing an alkali or alkaline-earth metallic oxide has a greater discharge coefficient of secondary electrons than a protective layer containing only magnesium oxide.

**Table 1**

| Deposition Method | Protective Layer | Discharge Coefficient of Secondary Electrons |
|---|---|---|
| E-beam | MgO | 0.33 |
| | MgO + Alkali metal | 0.53~0.60 |
| Sputtering | MgO | 0.40 |
| | MgO + Alkaline-earth metal | 0.56~0.62 |

Specifically, the metallic oxide may be selected from the group consisting of SrCaO, MgCaO, MgSrO and CsI. The metallic oxide, constituting the second protective layer 100b, may be located only on a part of the first protective layer 100a. More specifically, the metallic oxide may have the form of lumps distributed on the first protective layer 100a. The metallic oxide is patterned on the first protective layer 100a according to the pattern of transparent electrodes, to provide the first protective layer 100a with an uneven surface. Accordingly, while a gas discharge occurs in the plasma display panel, ultraviolet ions collide with the protective layer over an increased surface area of the protective layer, whereby the discharge amount of secondary electrons can be increased and a discharge start voltage can be lowered. This consequently has the effects of improving a discharge efficiency and restricting jitter characteristics. These effects can be more enhanced when the metallic oxide constituting the second protective layer 100b has a greater discharge coefficient of secondary electrons than that of magnesium oxide.

The metallic oxide, constituting the second protective layer 100b, may have the form of lumps distributed on the basis of the pattern of transparent electrodes in a panel. Here, in addition to protecting the transparent electrodes, the metallic oxide also has the function of converting vacuum ultraviolet rays having a wavelength of 147 nanometers, which is produced by a discharge gas such as xenon (Xe) during a discharge of the plasma display panel, into ultraviolet rays having a wavelength of 250 nanometers, and consequently, improving the brightness of the plasma display panel.

FIG. 2 is a perspective view illustrating the configuration of discharge cells included in the plasma display panel according to an embodiment of the present invention. Now, the embodiment of the plasma display panel according to the present invention will be described with reference to FIG. 2.

The plasma display panel according to the present embodiment includes an upper panel and a lower panel, which are arranged to face each other while interposing barrier ribs therebetween. The upper panel includes an upper substrate 70 having an image display surface, and sustain electrode pairs arranged on the upper substrate 70, each sustain electrode pair consisting of a pair of transparent electrodes 80a and 80b and a pair of bus electrodes 80a' and 80b'. The lower panel includes a lower substrate 10, and address electrodes 20 arranged on the lower substrate 10 to intersect the above described sustain electrode pairs. The upper panel and the lower panel are coupled parallel to each other with a predetermined distance therebetween.

To form a plurality of discharge spaces, i.e. discharge cells, the stripe type or well type barrier ribs 40 are arranged parallel to one another on the lower panel. The plurality of address electrodes 20 are arranged parallel to the barrier ribs, to generate vacuum ultraviolet rays by performing an address discharge. Red, Green, and Blue phosphors 50a, 50b, and 50c are applied onto an upper surface of the lower panel, to discharge visible rays for displaying an image during the address discharge. A lower dielectric layer 30 is formed between the address electrodes 20 and the phosphors 50a, 50b, and 50c, to protect the address electrodes 20.

An upper dielectric layer 90 is formed on the sustain electrode pairs, and in turn, the first protective layer 100a and the second protective layer 100b are formed on the upper dielectric layer 90 in sequence. The detailed characteristics of the first and second protective layers 100a and 100b are as described above. Here, although positive ions are produced while a discharge occurs in the discharge spaces, the first protective layer 100a, which is made of magnesium oxide, etc., protects the upper dielectric layer 90. Also, the second protective layer 100b, which is in contact with the discharge spaces, is made of magnesium oxide, etc., to achieve an improvement in discharge characteristics as described above.

FIGs. 3A and 3B are graphs illustrating a surface discharge voltage and an opposed discharge voltage of the plasma display panel according to the present invention.
FIG. 4A is a graph illustrating the jitter characteristics of the plasma display panel according to the present invention. FIG. 4B is a graph illustrating the cathode ray luminescence characteristics of a metallic oxide constituting the protective layer of the plasma display panel according to the present invention.

As shown in FIG. 3A, a conventional plasma display panel causes a surface discharge at approximately 320 volts, but the plasma display panel according to the present invention causes a surface discharge at 305 volts or less. Also, as shown in FIG. 3B, the conventional plasma display panel causes an opposed discharge at approximately 258 volts, but the plasma display panel according to the present invention causes an opposed discharge at 250 volts or less. Accordingly, the present invention has the effect of lowering a discharge start voltage, thereby lowering the consumption of electricity by the plasma display panel.

Discharge characteristics of the conventional plasma display panel having a film type protective layer and the plasma display panel of the present invention having a metallic oxide type protective layer will be represented in the following Table 2.

**Table 2**

| | Film | Metallic Oxide |
|---|---|---|
| Surface Discharge | 320 V | 303 V |
| Opposed Discharge | 258 V | 247 V |

As shown in FIG. 4A, the conventional plasma display panel having a film type protective layer has a discharge delay time of approximately 2 microseconds, but the plasma display panel according to the present invention has a discharge delay time of 1.2 microseconds or less. Here, the jitter characteristics of the film type protective layer of the conventional plasma display panel and the metallic oxide type protective layer of the plasma display panel according to the present invention will be represented in the following Table 3.

**Table 3**

| | Film | Metallic Oxide |
|---|---|---|
| T_{99.9} | 2.265 | 1.115 |
| T_{f} | 0.600 | 0.785 |
| T_{avg} | 0.982 | 0.928 |
| Sigma | 0.249 | 0.054 |
| T_{sc6z} | 2.477 | 1.252 |

It can be appreciated from the above Table 3 that the film type protective layer has a slightly faster formative time T_{f}, but other times are more shortened in the metallic oxide type protective layer, resulting in a reduction in the overall discharge delay time of the metallic oxide type protective layer. Such an improvement in jitter characteristics is accomplished by the fact that a metallic oxide contained in the second protective layer has a maximum cathode ray luminescence value within a wavelength region of 300 to 500 nanometers.

Hereinafter, a method for manufacturing a plasma display panel according to an embodiment of the present invention will be described. The method of the present embodiment is related to the manufacture of the plasma display panel having the above described configuration.

First, a first protective layer is deposited on a dielectric layer that was previously formed on an upper panel. Here, the first protective layer may be formed by any one method selected from among a spray method, a coating method, a chemical vapor deposition (CVD) method, an electronic beam (E-beam) method, an ion-plating method, a sol-gel method, a sputtering method, and the like. The first protective layer is formed close to the dielectric layer, to protect the dielectric layer from shock caused by positive ions, etc. To achieve the above described characteristics, the first protective layer preferably has a thickness of 100 to 1,000 nanometers. In the present exemplary embodiment, if the thickness of the first protective layer is less than 100 nanometers, there is a risk of an erroneous discharge. On the other hand, if the thickness of the first protective layer is more than 1,000 nanometers, it may cause problems in manufacturing processes and costs. The first protective layer contains magnesium oxide, and additionally, may contain the above described dopant. If the dopant is added, it has the effect of lowering a jitter value during an address discharge period. However, if the content of the dopant exceeds a predetermined value or more, it may disadvantageously increase the jitter value. Therefore, preferably, the doping of the dopant is performed within a range to reduce the jitter value to the maximum extent, and more preferable, the dopant is contained in the protective layer in an amount of 20 to 500 ppm.

Now, the deposition of the first protective layer using an electronic beam (E-beam) method will be described. First, a first source material as a constituent material of the first protective layer is prepared. As described above, the first source material consists of magnesium oxide and a slight amount of dopant, and the dopant is selected from the group consisting of Al, Cr, H₂, Si, Sc and Gd. Although the first source material may be provided as a single source material obtained by doping the above described dopant in magnesium oxide, the magnesium oxide and the dopant may be prepared separately. Subsequently, the above described first source material is heated at a high temperature, to deposit the first protective layer on the dielectric layer by use of a physical energy.

Then, the second protective layer is deposited on the first protective layer by any one method selected from a spray method, a coating method, a chemical vapor deposition (CVD) method, an electronic beam (E-beam) method, an ion-plating method, a sol-gel method, a sputtering method, and the like. Now, the deposition of the second protective layer using the chemical vapor deposition method will be described. The second protective layer has a feature of containing a single-crystal metallic oxide having a maximum cathode ray luminescence value within a wavelength region of 300 to 500 nanometers. The metallic oxide is obtained by supplying a gas-phase metallic element with 2 to 20 sccm of oxygen and 0 to 18 sccm of argon.

First, a second source material as a constituent material of the second protective layer is prepared. Here, the second source material consists of only magnesium oxide. The second protective layer is formed on the first protective layer by use of steam generated by heating the second source material. In this case, the magnesium oxide is deposited to have a single crystal structure. With the chemical vapor deposition method, the magnesium oxide in the second protective layer has a medium physical property of a layer and a crystal, and can reinforce the deposition strength of the second protective layer as compared to a spray method, etc.

FIG. 5 is a view illustrating an embodiment of a chemical vapor deposition apparatus according to the present invention. The embodiment of the chemical vapor deposition apparatus according to the present invention will be described hereinafter.

The chemical vapor deposition apparatus according to the present invention includes a chamber, a temperature regulator, and a controller. As shown in FIG. 5, the chamber 200 includes an inlet portion 210 for injecting a source material, etc. into the chamber 200, and an outlet portion 220 for discharging the source material, etc. to the outside. Also, although not shown in FIG. 5, the chamber 200 is provided with the temperature regulator for regulating the interior temperature of the chamber 200 and the controller for regulating the flow rates of a carrier gas and a reaction gas within the chamber 200.

After the upper panel of the plasma display panel formed with the first protective layer 100a is put into the above described chamber 200, the second protective layer 100b is formed via the chemical vapor deposition method. In this case, a carrier gas, a reaction gas, a precursor, and a source material are injected into the chamber 200. The source material is, for example, metal-alkoxide, to facilitate the growth of magnesium oxide crystals. The carrier gas may be nitrogen or hydrogen, and the reaction gas may be any one of oxygen, hydrogen, nitrogen, and argon.

In a process for forming the second protective layer on the first protective layer, nucleus generation sites are formed on the first protective layer, and a magnesium oxide single crystal is grown from each of the sites. Each magnesium oxide single crystal has an irregular shape, and thus, the overall protective layer has an uneven surface. In this case, the second protective layer preferably has a thickness of 100 to 1,500 nanometers. To satisfy the above described characteristics, preferably, the flow rates of the carrier gas and the reaction gas are regulated by the controller, and the interior temperature of the chamber is regulated by the temperature regulator.

The above described second protective layer may be deposited by a liquid phase deposition method, rather than the chemical vapor deposition method. Hereinafter, the deposition of the second protective layer using the liquid phase deposition method will be described.

First, the formation of the second protective layer using an alkali or alkaline-earth metallic oxide will be described.

First, as shown in FIG. 6, a second protective layer liquid is prepared by pre-mixing a solvent, a dispersant, and a single-crystal metallic oxide powder (S410). The metallic oxide may be an alkali or alkaline-earth metallic oxide. Here, 1 to 10 wt% of the single-crystal metallic oxide powder is mixed with 90 to 99 wt% of the solvent and the dispersant. The solvent may be an alcohol, glycol or diol, propylene glycol ether, propylene glycol acetate, ketone, butyl carbitol acetate (BCA), xylene, terpineol, texanol, water, or a mixture thereof. The dispersant may be acryl, epoxy, urethane, acrylic urethane, alkyd, poly amid polymer, poly carboxylic acid, or a mixture thereof.

Subsequently, the prepared second protective layer liquid is subjected to a milling process (S420). Here, the milling of the second protective layer liquid is performed by a milling machine.

The preparation of the second protective layer liquid is continued for 1 to 10 minutes at 2,000 to 4,000 rpm. The milling of the second protective layer liquid is continued for 10 to 60 minutes at 6,000 to 10,000 rpm. The solvent, the dispersant, and the single-crystal metallic oxide powder are mixed by stirring for a predetermined time (for example, for an hour), and are subjected to an ultrasonic distribution using an ultrasonic distributor, to thereby form the second protective layer liquid.

Next, the milled second protective layer liquid is applied onto the overall surface of the first protective layer by any one method selected from a spray coating method, a bar coating method, a screen printing method, and a green sheet method (S430). Thereafter, the second protective layer liquid, applied onto the first protective layer, is dried and fired (S440), to form the second protective layer (S450). Here, on the basis of the kind of the solvent, the drying is performed at a temperature of 100 to 200 degrees centigrade, and the firing is performed at a temperature of 400 to 600 degrees centigrade. Thereby, particles including the single-crystal metallic oxide powder remain irregularly, in the form of lumps, on the overall surface of the first protective layer, to form the second protective layer.

Hereinafter, a process for forming the second protective layer via the deposition of the single-crystal magnesium oxide powder will be described.

First, a solvent, a dispersant, and a single-crystal magnesium oxide (MgO) nano-powder are pre-mixed, to prepare a second protective layer liquid (S410). Here, 1 to 20 wt% of the single-crystal magnesium oxide nano-powder is mixed with 80 to 99 wt% of the solvent and the dispersant. The solvent may be an alcohol, glycol or diol, propylene glycol ether, propylene glycol acetate, ketone, butyl carbitol acetate (BCA), xylene, terpineol, texanol, water, or a mixture thereof. The dispersant may be acryl, epoxy, urethane, acrylic urethane, alkyd, poly amid polymer, poly carboxylic acid, or a mixture thereof.

Subsequently, the solvent, the dispersant, and the single-crystal magnesium oxide nano-powder are mixed by stirring for a predetermined time (for example, for an hour), and are subjected to an ultrasonic dispersion using an ultrasonic distributor, to thereby form the second protective layer liquid. Next, the second protective layer liquid is subjected to a milling process (S420). Here, the milling of the second protective layer liquid is performed by a milling machine. Next, the milled second protective layer liquid is applied onto the first protective layer by any one method selected from a screen printing method, a dispensing method, a photolithography method, and an ink-jet method (S430).

The second protective layer liquid, applied onto the first protective layer, is dried and fired (S440), to form the second protective layer (S450). Here, on the basis of the kind of the solvent, the drying is performed at a temperature of 100 to 200 degrees centigrade, and the firing is performed at a temperature of 400 to 600 degrees centigrade. Thereby, particles including the single-crystal metallic oxide nano-powder remain, in the form of lumps, on predetermined positions of the first protective layer, to form the second protective layer.

Other processes except for the above described protective layer forming process are identical to those included in a conventional plasma display panel manufacturing method.

First, after preparing an upper substrate by processing glass, two transparent electrodes (ITO) are formed on the upper substrate, and in turn, bus electrodes as auxiliary electrodes are deposited on certain positions of the respective electrodes, to form discharge cell sustain electrodes. Next, an upper dielectric layer is formed over the above electrodes, and in turn, a first protective layer and a second protective layer are formed on the dielectric layer in sequence.

The manufacture of a lower substrate comprises an operation for forming address electrodes on a glass substrate, an operation for forming a lower dielectric layer for the protection of the address electrodes, an operation for forming barrier ribs on an upper surface of the lower dielectric layer to divide discharge cells from one another, and an operation for forming a phosphor layer between the barrier ribs for discharging visible rays required for the display of an image.

Subsequently, a sealing material is applied onto the lower substrate formed with the address electrodes, to bond the lower substrate to the upper substrate. In this way, the manufacture of the plasma display panel is completed.

It will be apparent to those skilled in the art that various modifications and variations can be made in the present invention without departing from the scope of the invention. Thus, it is intended that the present invention covers the modifications and variations of this invention provided they come within the scope of the appended claims.

## Claims

1. A plasma display panel comprising a first panel and a second panel arranged to face each other while interposing barrier ribs therebetween, further comprising:
a first protective layer formed on a dielectric layer of the first panel; and
a second protective layer formed on the first protective layer and containing a metallic oxide having a maximum cathode ray luminescence value within a wavelength region of 300 to 500 nanometers.

2. The plasma display panel according to claim 1, wherein the metallic oxide is formed by supplying a gas-phase metallic element with 2 to 20 sccm of oxygen and 0 to 18 sccm of argon.

3. The plasma display panel according to claim 1, wherein the metallic oxide is a single-crystal magnesium oxide powder.

4. The plasma display panel according to claim 1, wherein a discharge delay time is 1.2 microseconds or less.

5. The plasma display panel according to claim 1, wherein a surface discharge start voltage is 305 volts or less, and an opposed discharge start voltage is 250 volts or less.

6. The plasma display panel according to claim 3, wherein the single-crystal magnesium oxide powder is formed on a part of the first protective layer.

7. The plasma display panel according to claim 3, wherein the single-crystal magnesium oxide powder has the form of lumps distributed on the first protective layer.

8. The plasma display panel according to claim 1, wherein the metallic oxide is an alkali or alkaline-earth metallic oxide.

9. The plasma display panel according to claim 8, wherein the metallic oxide is selected from the group consisting of SrCaO, MgCaO, MgSrO, and CsI.

10. The plasma display panel according to claim 1, wherein the metallic oxide is a powder having a particle size of 50 to 1,000 nanometers.

11. The plasma display panel according to claim 1, wherein the first protective layer has a thickness of 100 to 1,000 nanometers.

12. The plasma display panel according to claim 1, wherein the second protective layer has a thickness of 100 to 1,500 nanometers.

13. The plasma display panel according to claim 1, wherein the metallic oxide has a greater discharge coefficient of secondary electrons than that of magnesium oxide.

14. A method for manufacturing a plasma display panel comprising:
depositing a first protective layer on a dielectric layer of a first panel; and
depositing a second protective layer on the first protective layer, the second protective layer containing a single-crystal metallic oxide having a maximum cathode ray luminescence value within a wavelength region of 300 to 500 nanometers.

15. The method according to claim 14, wherein the single-crystal metallic oxide is formed by a vapor deposition.

16. The method according to claim 15, wherein the single-crystal metallic oxide is formed by supplying a gas-phase metallic element with 2 to 20 sccm of oxygen and 0 to 18 sccm of argon.

17. The method according to claim 14, wherein the deposition of the second protective layer comprises:
pre-mixing a solvent, a dispersant, and a single-crystal alkali or alkaline-earth metallic oxide powder, to prepare a second protective layer liquid;
milling the second protective layer liquid; and
applying the milled second protective layer liquid on the first protective layer, and drying and firing the second protective layer liquid.

18. The method according to claim 17, wherein the second protective layer liquid is prepared by mixing 1 to 10 wt% of the single-crystal alkali or alkaline-earth metallic oxide powder with 90 to 99 wt% of the solvent and the dispersant.

19. The method according to claim 17, wherein the solvent is alcohol, glycol or diol, propylene glycol ether, propylene glycol acetate, ketone, butyl carbitol acetate (BCA), xylene, terpineol, texanol, water, or a mixture thereof.

20. The method according to claim 17, wherein the dispersant is acryl, epoxy, urethane, acrylic urethane, alkyd, poly amid polymer, poly carboxylic acid (PCA), or a mixture thereof.

21. The method according to claim 17, wherein the application of the second protective layer liquid is performed by any one method selected from among a spray coating method, a bar coating method, a screen printing method, and a green sheet method.

22. The method according to claim 17, wherein the second protective layer liquid is dried at a temperature of 100 to 200 degrees centigrade, and is fired at a temperature of 400 to 600 degrees centigrade.

23. The method according to claim 14, wherein the deposition of the second protective layer comprises:
pre-mixing a solvent, a dispersant, and a single-crystal magnesium oxide nano-powder, to prepare a second protective layer liquid;
milling the second protective layer liquid; and
applying the milled second protective layer liquid on the first protective layer, and drying and firing the second protective layer liquid.

24. The method according to claim 23, wherein the second protective layer liquid is prepared by mixing 1 to 20 wt% of the single-crystal magnesium oxide nano-powder with 80 to 99 wt% of the solvent and the dispersant.

25. The method according to claim 23, wherein the mixing of the solvent, the dispersant, and the single-crystal magnesium oxide nano-powder is performed by stirring the mixture for a predetermined time or by an ultrasonic dispersion.

26. The method according to claim 23, wherein the application of the second protective layer liquid onto the first protective layer is performed by any one method selected from among a screen printing method, a dispensing method, a photolithography method, and an ink-jet method.

27. The method according to claim 14, wherein the second protective layer has the form of metallic oxide lumps distributed on the basis of a pattern of transparent electrodes on the first panel.

28. A method for manufacturing magnesium oxide comprising:
preparing magnesium gas; and
supplying the magnesium gas with oxygen gas and argon gas, to form a magnesium oxide single crystal.

29. The method according to claim 28, wherein the oxygen gas is supplied at a flow rate of 2 to 20 sccm, and the argon gas is supplied at a flow rate of 0 to 18 sccm.
